

## UNITED STATES PATENT OFFICE.

JAMES H. GRAVELL, OF ELKINS PARK, PENNSYLVANIA, ASSIGNOR TO AMERICAN CHEMICAL PAINT COMPANY, OF AMBLER, PENNSYLVANIA, A CORPORATION OF DELAWARE.

## METAL CLEANING.

No Drawing.

Application filed June 22, 1926. Serial No. 117,876.

This invention relates to the art of cleaning ferrous metals and although generally useful in that art, it is particularly directed to preparing steel for painting.

5 Steel is prepared for painting by treating it with an admixture of a metal etching acid and a material for causing the acid to wet even an oily surface,—an admixture of alcohol and phosphoric acid is a typical example. After the cleaner has performed its function it is removed along with the products of its reaction by washing the surface with water. The surface is then dried or 10 is permitted to dry, and is then ready for receiving the priming coat of the protective coating which may be paint, varnish, lacquer or japan, and the like.

It is found that after the drying operation, the metal is stained due to the formation 20 of iron oxide which not only mars the surface but acts to prevent the priming coat or protective coating from contacting with the true metallic surface.

One object of the invention is to provide 25 a method of cleaning steel which reduces or obviates the staining of the work to such an extent that it becomes commercially negligible. Further objects of this invention are to provide a cleaning method that will not 30 cause rust; a cleaning method that will permit the cleaned metal to remain for long periods without a subsequent protective coating and without rusting; a cleaning method which simultaneously cleans and provides a 35 protective coating. It is also an object of this invention to provide a cleaner for steel whose use will not cause the metal to rust or tarnish.

I have discovered that if steel is metallically plated while it is being cleaned, staining in 40 the washing step of the cleaning process is avoided. I have found that arsenic is best suited for my purpose, as a very thin coating or film of it suffices for my purpose, and 45 under proper conditions it dissolves readily in suitable acid admixtures, and in addition it is electro negative to steel, and hence plates out of solution by simple immersion or contact and therefore does not require recourse 50 to the aid of an electric current.

Though I may dissolve arsenic in the form 55 of arsenious oxide directly in my acid admixture, I prefer to first dissolve the arsenious oxide in an alkaline solution and then to introduce the proper amount of this alkaline

solution into my admixture, as by this method the solution of the arsenic in my admixture is more rapid. A suitable alkaline solution of arsenic may be made by mixing:

|                  |    |             |
|------------------|----|-------------|
| Water            | 60 | .92 gallons |
| Sodium hydroxide | 65 | 1.33 pounds |
| Arsenious oxide  | 70 | 1.66 pounds |

My cleaner primarily consists of a metal etching acid, a material for causing the acid to wet an oily surface and a chemical for creating or providing a metallic coating of arsenic. I find phosphoric acid produces good results. The material for causing the acid to wet an oily surface may be methyl alcohol, ethyl alcohol, denatured alcohol, butyl alcohol, propyl alcohol, amyl alcohol, acetone, ethyl acetate, methyl-ethyl ketone, fusel oil and the like. I consider that denatured alcohol either alone or mixed with butyl alcohol produces the best results.

A suitable admixture for practicing my invention is made by using:

|                           | Gallons. | 80  |
|---------------------------|----------|-----|
| Water                     | 80       | .50 |
| Phosphoric acid (85%)     | 85       | .33 |
| Denatured alcohol         | 90       | .20 |
| Butyl alcohol             | 95       | .05 |
| Alkaline arsenic solution | 100      | .02 |

The metal to be treated according to my method may be befooled by rust, oil, dirt, hand marks, acid runs, soldering fluid or any of those objectionable materials which are apt to cause a development of defects in applied finishes. When manipulated according to my process, my cleaner removes these objectionable materials and leaves the cleaned surface free from tarnish and in a suitable condition for receiving the protective coating.

To carry out the process, I apply the described admixture to the metal to be cleaned in any suitable manner, but preferably with a brush; I allow the admixture sufficient time 100 to act on the surface, assisting the action in the meantime if necessary by scrubbing with an abrasive; when the proper degree of cleanliness has been obtained, the spent cleaner along with the deleterious products of its reaction are removed. This removing step in the process is best accomplished by washing the metal with water. The water may be either cold or hot but preferably first cold 105 and then hot, thus leaving the metal heated 110

and causing it to dry quickly, by evaporation. The drying may be assisted by wiping with cloths or blowing off with a jet of air.

The action of my cleaner is such that a thin coating or film of metallic arsenic is deposited on the cleaned metal which acts to prevent the formation of tarnish during the drying step in the process.

I claim:

10 1. A ferrous metal cleaner comprising an admixture of phosphoric acid and a material adapted to remove oil from an oily surface in proportions fixed by the fact that the more acid the quicker the removal of oxide and the 15 more of the material the better the removal

of oil, and a compound of arsenic in proportion fixed by the possibility of getting it into the solution and adapted by contact to plate out a film of metallic arsenic on the ferrous metal surface.

20 2. A cleaner for ferrous metals comprising an admixture of metal etching acid and a material adapted to remove oil from an oily surface in proportions substantially as described, and a compound of arsenic in substantially the proportion described and adapted by contact to deposit a film of metallic arsenic on the ferrous metal which film opposes tarnish during drying.

25 JAMES H. GRAVELL.